

Patented May 30, 1944

2,349,817

## UNITED STATES PATENT OFFICE

2,349,817

POLYCARBOXYLIC ACID SALTS IN LUBE  
OIL COMPOUNDING

Bruce B. Farrington, James O. Clayton, and Dorr H. Etzler, Berkeley, Calif., assignors to Standard Oil Company of California, San Francisco, Calif., a corporation of Delaware

No Drawing. Application March 8, 1940,  
Serial No. 322,946

18 Claims. (Cl. 252—39)

This invention relates to new and useful compositions of matter and to methods of preparing the same. In particular, it relates to compositions comprising hydrocarbons of the lubricating oil class, in major part, in which are dissolved or suspended minor amounts of certain metal salts of organic aliphatic carboxylic acids, either alone or in admixture with other compounding agents of the same or different type.

It has long been the desire of the lubricating oil compounding art to obtain an oil, particularly of petroleum origin, which alone or with the addition of relatively small amounts of compounding agents, would resist deterioration or degradation when subjected for long periods of time to high temperatures and pressures, in the presence of metals, air or oxygen, or hydrocarbon partial combustion products. Deterioration of the character referred to here manifests itself in diverse effects, dependent upon the nature and degree of refinement of the hydrocarbon oil and upon the environment to which it is subjected, but reference may be made to Diesel engine piston ring sticking, in which the exposure of a lubricating oil to such temperatures as 425°—650° F., in the presence of oxidizing combustion gases at pressures as high as 750—1150 lbs./sq. in., causes the deposition of oil degradation products of such a cementitious character as to effectively take piston rings out of service; to the deposition of "sludge" from automobile crank case oils, apparently as the result of oxidation and/or polymerization phenomena; and to the corrosion of metal bearing surfaces, apparently as a result of phenomena which cause the formation of organic acidic products. This situation

is aggravated by the fact that improvements in the mechanical arts have brought about increasing severity in the conditions to which hydrocarbon oils are subjected, and by the fact that 5 oil compounding designed to effect a stability in one direction often brings about a marked instability in another.

It has been found that the addition to a lubricating oil of small amounts of a metal salt of 10 an aliphatic carboxylic acid, carrying a substituted or unsubstituted carboxylic acid group in addition to the salt-forming carboxylic acid group, brings about an improved stability in hydrocarbon oils when the same are subjected to 15 high temperatures and/or pressures in the presence of oxygen and metals; such acids correspond in general to the type  $\text{HOOC}-(\text{CH}_2)_n-\text{COOH}$ , in which  $n$  may be zero or a whole number, generally from 1 to 8 inclusive, although compounds 20 in which  $n$  is greater than 8 are fully operative, in which there may or may not be alkyl, aryl, aralkyl or carbocyclic hydrocarbon substitution to increase oil solubility. It has further been found that still greater improvement of the desired sort is brought about when, in the metal salts of acids of the type  $\text{HOOC}-(\text{CH}_2)_n-\text{COOH}$  25 ( $n=0-8$ ), if  $n$  is greater than 1 or 2, certain polar group substitution is effected in a position alpha, beta, gamma, delta or even epsilon to the carbon atom of the salt-forming carboxylic acid group, the effectiveness for the desired purpose decreasing in the order of position as recited.

For the purposes of this invention the term 30 "polar group" is defined as including the following radicals:

| Name                         | Formula                    | Name                      | Formula                        |
|------------------------------|----------------------------|---------------------------|--------------------------------|
| Carboxylic acid              | $-\text{COOH}$             | Alkamino or arylamino     | $-\text{NHR}$                  |
| Metallo-carboxyl             | $-\text{COOM}$             | Dialkamino or diarylamino | $-\text{NR}_2$                 |
| Esterified carboxyl          | $-\text{COOR}$             | Azo                       | $-\text{N}=\text{N}-$          |
| Hydroxyl                     | $-\text{OH}$               | Hydrazo                   | $-\text{NHNH}-$                |
| Vinylene                     | $-\text{CH}=\text{CH}-$    | Hydrazono                 | $-\text{N}-\text{NH}_2$        |
| Amino                        | $-\text{NH}_2$             | Triazeno                  | $-\text{NNN}-$                 |
| Ethyneylene                  | $-\text{C}\equiv\text{C}-$ | Triazo                    | $-\text{NNN}$                  |
| Alkoxy or aryloxy            | $-\text{OR}$               | Cyano                     | $-\text{CN}$                   |
| Metallo-oxy                  | $-\text{OM}$               | Isocyano                  | $-\text{NC}$                   |
| Oxo or keto                  | $=\text{O}$                | Cyanate                   | $-\text{OCN}$                  |
| Carbamyl                     | $-\text{CO}(\text{NH}_2)$  | Isocyanate                | $-\text{NOO}$                  |
| Alkyl or aryl thiolecarboxyl | $-\text{COSR}$             | Thiocyanate               | $-\text{SCN}$                  |
| Alkyl or aryl thionocarboxyl | $-\text{CSO R}$            | Isothiocyanate            | $-\text{SNC}$                  |
| Mercapto                     | $-\text{SH}$               | Nitroso                   | $-\text{NO}$                   |
| Alkyl or arylthio            | $-\text{SR}$               | Nitro                     | $-\text{NO}_2$                 |
| Thiono                       | $-\text{S}$                | Isonitroso                | $=\text{NOH}$                  |
| Dithio                       | $-\text{SS}$               | Hydroxamino               | $-\text{NHOH}$                 |
| Sulfinyl                     | $-\text{SO}$               | Azoxy                     | $-\text{NON}-$                 |
| Sulfonyl                     | $-\text{SO}_2$             | Isonitro                  | $-\text{NOO}$                  |
| Imino                        | $-\text{NH}$               | Phosphino                 | $-\text{PH}$ ; or $=\text{PH}$ |

| Name                         | Formula                          | Name                        | Formula                   |
|------------------------------|----------------------------------|-----------------------------|---------------------------|
| Phosphoro...                 | —PO                              | Phosphazo...                | —PN—                      |
| Phospho...                   | —PO <sub>2</sub>                 | Phosphoro...                | —PP—                      |
| Alkyl or aryl phosphate...   | —OP(O R) <sub>2</sub>            | Phosphoarseno...            | —PAs—                     |
| Alkyl or aryl phosphite...   | —O P(O R) <sub>2</sub>           | Arsino...                   | —AsH <sub>2</sub> or =AsH |
| Silicyl...                   | —SiH <sub>3</sub>                | Arsenos...                  | —AsO                      |
| Silicylene...                | —SiH <sub>2</sub>                | Arso...                     | —AsO <sub>2</sub>         |
| Alkyl or aryl silicono...    | —SiO R                           | Alkyl or aryl arsenate...   | —OAsO(O R) <sub>2</sub>   |
| Alkyl or aryl sulfino...     | —SO <sub>2</sub> R               | Alkyl or aryl arsenite...   | —OAs(O R) <sub>2</sub>    |
| Alkyl or aryl sulfo...       | —SO <sub>3</sub> R               | Alkyl or aryl arsono...     | —AsO(O R) <sub>2</sub>    |
| Alkyl or aryl sulfamino...   | —NHSO <sub>3</sub> R             | Alkyl or aryl arsonico...   | —AsO O R                  |
| Sulfamyl...                  | —SO <sub>2</sub> NH <sub>2</sub> | Arseno...                   | —AsAs—                    |
| Sulfonamido...               | —SO <sub>2</sub> NH—             | Stibino...                  | —SbH <sub>2</sub> or =SbH |
| Selenyl...                   | —SeH                             | Stiboso...                  | —SbO                      |
| Alkyl or aryl selenyl...     | —SeR                             | Stibo...                    | —SbO <sub>2</sub>         |
| Seleno...                    | —Se                              | Alkyl or aryl antimonate... | —OSbO(O R) <sub>2</sub>   |
| Seleninyl...                 | —SeO                             | Alkyl or aryl stibono...    | —SbO(O R) <sub>2</sub>    |
| Selenonyl...                 | —SeO <sub>2</sub>                | Alkyl or aryl stibinico...  | —SbO O R                  |
| Alkyl or aryl selenino...    | —SeO(O R)                        | Antimono...                 | —SbSb—                    |
| Alkyl or aryl selenono...    | —SeO <sub>2</sub> (O R)          | Stibarseno...               | —SbAs—                    |
| Selenociano...               | —SeCN                            | Bismuthino...               | —BiH <sub>2</sub> or =BiH |
| Telluryl...                  | —TeH                             | Boryl...                    | —BO                       |
| Alkyl or aryl telluryl...    | —TeR                             | Alkyl or aryl borate...     | —OB(O R) <sub>2</sub>     |
| Telluro...                   | —Te                              | Iodoso...                   | —OSi(O R) <sub>2</sub>    |
| Alkyl or aryl phosphonite... | —P(O R) <sub>2</sub>             | Stannyl...                  | —IO                       |
| Alkyl or aryl phosphonate... | —PO(O R) <sub>2</sub>            | Iodoxy...                   | —SnH <sub>3</sub>         |
| Alkyl or aryl phosphinite... | —POR                             |                             | —IO <sub>2</sub>          |
| Alkyl or aryl phosphinate... | —POO R                           |                             |                           |

In the above polar group representations, R represents an alkyl, aryl or aralkyl radical. It is to be particularly noted that the simple halogeno groups (—Cl, —Br and —I) are not included here, because of the ease with which these groups split off and because of the extreme corrosivity and general reactivity of the halogen acids thus formed.

The metals whose substituted carboxylic acid salts are useful for the purposes of the invention may have valences from one to four, inclusive, and the salts of potassium, calcium, magnesium, aluminum, chromium, cobalt, lead, manganese, tin and zinc have been found of particular utility.

Among the aliphatic carboxylic acids whose metal salts are suitable in the practice of the invention and which correspond to the structure HOOC—(CH<sub>2</sub>)<sub>n</sub>—COOH (n=0-8 or a higher whole number) there may be mentioned: the oxalic acid series, including oxalic acid itself; malonic acid; isosuccinic or methylmalonic acid and its alkyl homologues such as ethylmalonic, dimethylmalonic, propyl- and iso-propylmalonic, methylethylmalonic, n-butyethylmalonic, isobutyethylmalonic, sec-butylmalonic, propylmethylmalonic, isopropylmethylmalonic, diethylmalonic, pentylmalonic, dipropylmalonic and cetylmalonic acids; succinic acid; the mono-alkylic succinic acids such as methylsuccinic, ethylsuccinic and iso-propylsuccinic; the symmetrical dialkylic succinic acids including symmetrical dimethylsuccinic, symmetrical methylethylsuccinic, symmetrical methylisopropylsuccinic, symmetrical diethylsuccinic and analogous higher alkylic homologues; the unsymmetrical dialkylic succinic acids such as unsymmetrical dimethylsuccinic, trimethyl- and tetramethylsuccinic acids; glutaric acid;  $\alpha$ -methylglutaric acid;  $\beta$ -methyl- and  $\beta$ -ethylglutaric acids; the di- and tri-alkylic glutaric acids such as  $\alpha,\alpha$ -dimethylglutaric,  $\alpha,\alpha$ -diethylglutaric,  $\alpha,\beta$ -dimethylglutaric, unsymmetrical  $\alpha,\alpha$ -dimethylglutaric,  $\beta,\beta$ -dimethylglutaric and the higher alkylic homologues of these acids;  $\alpha,\alpha,\alpha$ -trimethylglutaric acid; adipic acid;  $\alpha$ -methyl- and  $\alpha$ -ethyladipic acids;  $\beta$ -methyladipic acid;  $\alpha,\alpha$ -diethyl- and  $\alpha,\alpha$ -dimethyl adipic acids; pimelic acid and the alkylic pimelic acids including  $\alpha$ -,  $\beta$ -, and  $\gamma$ -methylpimelic,  $\alpha,\alpha$ -dimethylpimelic and  $\alpha,\beta,\alpha$ -trimethylpimelic acids; suberic acid and the alkylic suberic acids; and sebacic and the alkylic sebacic acids. Representative of these aliphatic acids in which one

vinylene group is the polar group referred to as augmenting the desired effects in the employment of suitable metal salts, for the purposes of the invention, may be mentioned: the alkylene malonic acids such as methylenemalonic acid, CH<sub>2</sub>:C(COOH)<sub>2</sub>; isopropylmalonic acid and allylmalonic acid, CH<sub>2</sub>:CH.CH<sub>2</sub>.CH(COOH)<sub>2</sub>; fumaric acid; maleic acid; mesaconic acid; citraconic acid; itaconic acid; glutaconic acid; teraconic acid and hydromuconic acid, together with the alkylic and dialkylic homologues of these olefine dicarboxylic acids. As representative of suitable acids in which two vinylene polar groups appear may be mentioned diallylmalonic acid, (CH<sub>2</sub>:CH.CH<sub>2</sub>)<sub>2</sub>C(COOH)<sub>2</sub>; muconic acid; and di-isovaleralglutaric acids. Representative of suitable acids in which the ethylene group is the polar group which makes the metal polycarboxylic acid salts especially suitable for the purposes of the invention, may be noted glutinic acid and diacetylenedicarboxylic acid. Examples of suitable acids in which a carboxylic group is the polar radical referred to as desirable are the paraffin tricarboxylic acids such as isobutane- $\alpha,\alpha,\beta$ -tricarboxylic acid, tricarballylic acid and  $\alpha,\alpha,\beta$ -trimethyltricarballylic or camphoronic acid, and the alkylic homologues thereof; and the olefine tricarboxylic acids such as aconitic acid and its isomers aceconitic and citraconic acids. Representative of suitable acids in which one or more hydroxy groups are the polar radicals referred to as especially beneficial are tartronic or oxymalonic acid and the several alkylic tartronic acids such as methyltartronic or isomalic acid, ethyltartronic, propyl- and isopropyltartronic; the  $\gamma$ -oxyalkylic malonic acids; malic acid and its homologues, for example  $\alpha$ -oxypyrotartaric acid,  $\beta$ -methylmalic acid,  $\alpha,\beta$ -methylmethylic acid, isopropylmalic acid and the paraconic acids;  $\alpha$ -oxyglutaric acid;  $\beta$ -oxyglutaric acid;  $\alpha$ -hydroxyadipic and  $\alpha$ -hydroxysebacic acid; the isomeric tartaric acids; citric acid; and dioxytartaric acid. The polar substituted derivatives of various of these and other aliphatic carboxylic acids, generally partially esterified, in the form of their metal salts, will be referred to below in more detailed exemplification of the practice of the process of the invention. As aforesaid, polar substitution of the character indicated, most suitably in the alpha, beta and gamma positions, and less suitably in the delta, epsilon, etc., positions, relative to the salt-forming carboxyl carbon atom, in the

enumerated order of preference, is especially beneficial for the purposes of the invention.

#### EXAMPLES—SET I

Among the beneficial effects which flow from the incorporation of a metal salt or a mixture of metal salts of the above described aliphatic acids in a hydrocarbon oil of the lubricating oil class is the prevention of piston ring sticking, or its marked postponement, under very severe motor conditions, as for example in Diesel engine or in aircraft spark or compression ignition engine operations.

In the tests whose results are summarized in Table I, a single cylinder Lauson gasoline spark-ignition engine, 2½ inch bore and 2½ inch stroke, loaded with fan dynamometers, was operated under extremely severe conditions, designed to develop fully the tendency of the crankcase lubricant to deteriorate with gum formation and piston ring sticking: operation was at 1600 R. P. M.; engine jacket temperature was maintained at 375° F.; crankcase oil temperature was maintained at 220° F.; at periods of 15 hours the operations were interrupted and the condition of the piston rings determined. In Table I, the base oil referred to as "Western 30" was an acid-refined lube stock of California origin; A. P. I. gravity 21.4°; viscosities at 100° and 210°, 622 seconds and 56.6 seconds, respectively, Saybolt Universal. To this base oil were added the various salts in the amounts indicated, by weight. The base or uncompounded oil referred to as "Pennsylvania 30" was a solvent refined stock of Pennsylvania origin, A. P. I. gravity 28.6°; viscosities at 100° and 210° F. of 519 and 66 seconds, respectively, Saybolt Universal.

of the cadmium-silver and copper-lead types. This diminution in corrosivity is particularly marked upon the incorporation in the hydrocarbon oils of metal salts of those aliphatic carboxylic acids corresponding to the type



( $n=0-8$  or a higher whole number) in which a polar group or radical as above exemplified is substituted for a hydrogen atom attached to a carbon atom in close proximity to the carbon atom of the salt-forming carboxylic acid radical—preferably in the alpha position, less preferably in the beta position and of decreasing desirability and effectiveness in the gamma, delta, epsilon, etc., positions, in the order named.

In the tests whose results are summarized in Tables II, thin sheets of the indicated bearing metals were cut into strips (copper-lead,  $\frac{1}{16}$ " x  $1\frac{3}{4}$ " x  $\frac{3}{32}$ "; cadmium-silver,  $\frac{1}{2}$ " x  $1\frac{3}{8}$ " x  $\frac{1}{16}$ "), and these strips were immersed in the exemplified oils carried in 2" x 20" glass test tubes; these test tubes were carried in an oil bath maintained at 300° F.  $\pm 1$ ° F. Each test tube contained approximately 300 cc. of oil, and air was bubbled through each tube at the rate of 10 liters per hour. At the end of each of three 24-hour periods, the strips were removed from the oils, washed with petroleum ether and carefully wiped with a soft cotton cloth; weight losses of the strips were measured in connection with the weight of each individual strip. The duration of the tests was 72 hours, and the weight losses tabulated below are those found at the end of the 72-hour period, except as indicated; the losses reported, however, represent the averages of at least two and sometimes more duplicate or check cor-

TABLE I  
*Prevention or postponement of piston ring sticking*

| Example | Oil                                                                       | Hours to cause ring sticking | Relative ring slot cleanliness | Relative piston cleanliness |
|---------|---------------------------------------------------------------------------|------------------------------|--------------------------------|-----------------------------|
| 1.      | Western 30.                                                               | 30                           | Poor.                          | Poor.                       |
| 2.      | +0.28% potassium cetyl tartrate.                                          | 60+                          | Good.                          | Good.                       |
| 3.      | +0.42% magnesium cetyl tartrate.                                          | 60+                          | Fair.                          | Fair.                       |
| 4.      | +0.57% aluminum cetyl tartrate.                                           | 60+                          | Poor.                          | Poor.                       |
| 5.      | +0.50% calcium cetyl tartrate.                                            | 120+                         | Very good.                     | Very good.                  |
| 6.      | +0.20% calcium cetyl mucate.                                              | 60+                          | Poor.                          | Poor.                       |
| 7.      | +0.34% potassium cetyl citrate.                                           | 120                          | Good.                          | Fair.                       |
| 8.      | +0.28% magnesium cetyl citrate.                                           | 60+                          | Fair.                          | Poor.                       |
| 9.      | +0.52% aluminum cetyl citrate.                                            | 60+                          | Good.                          | Fair.                       |
| 10.     | +0.50% calcium dicetyl citrate.                                           | 120+                         | Good.                          | Good.                       |
| 11.     | +0.63% calcium $\alpha$ -eicosyltartrate.                                 | 60+                          | Fair+                          | Good.                       |
| 12.     | +0.18% calcium cetyl oxalate.                                             | 120                          | Fair.                          | Poor.                       |
| 13.     | +0.50% calcium cetyl succinate.                                           | 90                           | Fair.                          | Fair+.                      |
| 14.     | +0.50% calcium cetyl malate.                                              | 105+                         | Good.                          | Good.                       |
| 15.     | +0.50% calcium $\alpha$ -cetylmalonate.                                   | 120                          | Good.                          | Fair.                       |
| 16.     | +0.50% calcium $\alpha$ -cetylsuccinate.                                  | 75                           | Fair.                          | Poor.                       |
| 17.     | +0.34% calcium $\alpha$ -eicosenylsuccinate.                              | 90                           | Fair+                          | Poor.                       |
| 18.     | +0.15% calcium cetyl sebacate.                                            | 120+                         | Good.                          | Fair.                       |
| 19.     | +0.40% calcium cetyl $\alpha$ -aminosuccinate.                            | 60                           | Fair.                          | Poor.                       |
| 33.     | +0.50% calcium cetylphenate+0.50% calcium cetyl tartrate.                 | 60+                          | Very good.                     | Very good.                  |
| 34.     | +0.50% calcium cetylphenate+0.50% calcium dicetyl citrate.                | 60+                          | Very good.                     | Very good.                  |
| 35.     | +0.50% calcium cetylphenate+0.25% calcium dicetyl citrate.                | 60+                          | Very good.                     | Very good.                  |
| 36.     | +0.50% calcium cetylphenate+0.50% calcium $\alpha$ -eicosyltartrate.      | 90+                          | Very good.                     | Very good.                  |
| 42.     | +0.50% calcium cetylphenate+0.50% calcium $\alpha$ -eicosenylsuccinate.   | 120+                         | Very good.                     | Very good.                  |
| 44.     | +0.50% calcium cetylphenate+0.50% calcium cetyl $\alpha$ -aminosuccinate. | 60                           | Fair.                          | Fair.                       |
| 74.     | Pennsylvania 30.                                                          | 60+                          | Very good.                     | Very good.                  |
| 76.     | +0.50% calcium cetyl tartrate.                                            | 30                           | Poor.                          | Poor.                       |
|         | +0.50% calcium cetylphenate+0.50% calcium dicetyl citrate.                | 60+                          | Good.                          | Poor.                       |
|         |                                                                           | 60+                          | Very good.                     | Very good.                  |

NOTE: A plus sign (+) following a stated number of hours in the antepenultimate column indicates free rings at the conclusion of a test of the stated hours' duration.

#### EXAMPLES—SET II

Among the further benefits to be derived from the addition of the metal salts of the invention to hydrocarbon lubricating oils is a decreased corrosivity toward bearing metals, particularly those

erosion tests under these conditions. In connection with the results reported in Table II, attention is directed to those oils compounded by the addition of agents other than those of the invention (oils A, B, C, etc.), in which the compound-

ing, while perhaps of benefit in respect to some property of the oil, is of definitely deleterious effect in respect to the corrosivity of the oil toward bearing metals. Attention is additionally directed to such compounded oils (within the example bracket 32-73) to which have been added, as further compounding agents, the metal salts herein particularly described, wherein it appears that the increased corrosivity due to the original compounding has been prevented or inhibited by the agents of the invention.

TABLE II  
Reduction of corrosivity to bearing metals

| Example | Oil                                                                          | Weight loss in mgms., 72 hrs. |       |
|---------|------------------------------------------------------------------------------|-------------------------------|-------|
|         |                                                                              | Cu-Pb                         | Cd-Ag |
| 1.      | Western 30.                                                                  | 13.9                          | 0.4   |
| 2.      | +0.28% potassium cetyl tartrate.                                             | 1.3                           | 0.1   |
| 4.      | +0.42% magnesium cetyl tartrate.                                             | 2.0                           | 0.3   |
| 5.      | +0.50% calcium cetyl tartrate.                                               | 1.3                           | 0.5   |
| 6.      | +0.20% calcium cetyl mucate.                                                 | 1.6                           | 0     |
| 7.      | +0.34% potassium cetyl citrate.                                              | 8.5                           | 0.4   |
| 8.      | +0.28% magnesium cetyl citrate.                                              | 2.1                           | 0     |
| 9.      | +0.52% aluminum cetyl citrate.                                               | 5.5                           | 0.5   |
| 10.     | +0.50% calcium dicetyl citrate.                                              | 2.6                           | 1.4   |
| 11.     | +0.63% calcium $\alpha$ -eicosyltartrate.                                    | 5.0                           | 0.9   |
| 12.     | +0.18% calcium cetyl oxalate.                                                | 1.2                           | 0     |
| 13.     | +0.50% calcium cetyl malate.                                                 | 3.7                           | 0.1   |
| 14.     | +0.50% calcium cetyl maleate.                                                | 2.0                           | 0     |
| 15.     | +0.50% calcium $\alpha$ -cetylmalonate.                                      | 9.8                           | 0.3   |
| 16.     | +0.50% calcium $\alpha$ -cetenylysuccinate.                                  | 1.1                           | 0.3   |
| 17.     | +0.34% calcium $\alpha$ -eicosenylsuccinate.                                 | 1.6                           | 0.1   |
| 18.     | +0.15% calcium cetyl sebacate.                                               | 7.1                           | 1.0   |
| 20.     | +0.16% calcium cetyl $\alpha$ -aminosuccinate.                               | 6.3                           | 0     |
| 21.     | +0.78% calcium cetyl malonate.                                               | 3.4                           | 0.1   |
| 22.     | +0.50% calcium cetyl $\alpha$ -mercaptosuccinate.                            | 11.1                          | 0.8   |
| 23.     | +0.50% calcium cetyl fumarate.                                               | 14.6                          | 1.5   |
| 33.     | +0.50% calcium cetylphenate+0.50% calcium cetyl tartrate.                    | 2.0                           | 0.2   |
| 34.     | +0.50% calcium cetylphenate+0.50% calcium dicetyl citrate.                   | 9.6                           | 1.3   |
| 35.     | +0.50% calcium cetylphenate+0.25% calcium dicetyl citrate.                   | 6.1                           | 0.1   |
| 42.     | +0.50% calcium cetylphenate+0.50% calcium $\alpha$ -eicosenylsuccinate.      | 40.7                          | 6.0   |
| 44.     | +0.50% calcium cetylphenate+0.50% calcium cetyl $\alpha$ -aminosuccinate.    | 11.8                          | 6.0   |
| 45.     | +0.50% calcium cetylphenate+0.50% calcium cetyl $\alpha$ -mercaptosuccinate. | 11.1                          | 0.8   |
| 56.     | +0.25% calcium cetylphosphate+0.50% calcium dicetyl tartrate.                | 1.3                           | 0.2   |
| A.      | +0.50% calcium stearate.                                                     | 131.9                         | 180.5 |
| B.      | +1.0% aluminum dinaphthenate.                                                | 67                            | 113   |
| C.      | +1.0% magnesium naphthenate.                                                 | 139                           | 119   |
| D.      | +1.0% calcium cetylphenate.                                                  | 126                           | 12.1  |
| 74.     | Pennsylvania 30.                                                             | 24.5                          | 1.6   |
| 75.     | +0.50% calcium cetyl tartrate.                                               | 1.3                           | 0.2   |
| 77.     | +0.50% calcium cetyl citrate.                                                | 18.7                          | 14.2  |
| 78.     | +0.50% calcium cetyl $\alpha$ -mercaptosuccinate.                            | 7.1                           | 0.0   |
| F.      | +0.50% calcium cetylphenate.                                                 | 20.7                          | 2.2   |
| G.      | +0.75% calcium cetylphenate.                                                 | 63.5                          | 47.6  |
| I.      | +0.10% calcium ricinoleate.                                                  | 166.6                         | 215.4 |
| J.      | +0.50% calcium $\alpha$ -bromostearate.                                      | 135.2                         | 222   |
| K.      | +1.0% aluminum dinaphthenate (24 hrs.)                                       | 125.7                         | 111.7 |
|         |                                                                              | 42.8                          | 28.6  |

#### EXAMPLES—SET III

A still further benefit to be derived from the addition of the metal salts of the invention to hydrocarbon oils, particularly noticeable in the case of salts of those acids carrying polar substituents as described, is a marked lessening of color instability upon exposure of the oils of the invention to heat, in the absence of air or metals.

In the tests whose results are summarized in Table III, samples of the exemplified oils were held, in glass, at 300° F. for 6 hours. The oils were cooled at the end of this period of time and their colors measured, for comparison with the un compounded base oil stocks; A. S. T. M. 75

colors, Method D155-34T, were recorded in all cases.

TABLE III  
Color stability

| Example | Oil                                                                                     | Color after heating | Color increase |
|---------|-----------------------------------------------------------------------------------------|---------------------|----------------|
| 10      | Western 30.                                                                             | 3 1/2 dil.          | 6              |
| 1       | +0.28% potassium cetyl tartrate.                                                        | 4 1/2               | 1/2            |
| 2       | +0.42% magnesium cetyl tartrate.                                                        | 7                   | 2+             |
| 3       | +0.57% aluminum cetyl tartrate.                                                         | 6                   | 1 1/2          |
| 4       | +0.50% calcium cetyl tartrate.                                                          | 4 1/2               | 1              |
| 5       | +0.20% calcium cetyl mucate.                                                            | 3 dil.              | 4              |
| 6       | +0.34% potassium cetyl citrate.                                                         | 6                   | 1 1/2          |
| 7       | +0.28% magnesium cetyl citrate.                                                         | 5                   | 1 1/2+         |
| 8       | +0.52% aluminum cetyl citrate.                                                          | 4                   | 1/2+           |
| 9       | +0.50% calcium dicetyl citrate.                                                         | 4                   | 1              |
| 10      | +0.63% calcium $\alpha$ -eicosyltartrate.                                               | 4                   | 1-             |
| 11      | +0.18% calcium cetyl oxalate.                                                           | 6                   | 3              |
| 12      | +0.50% calcium cetyl succinate.                                                         | 4 1/2               | 1+             |
| 13      | +0.50% calcium cetyl malate.                                                            | 4 1/2               | 1              |
| 14      | +0.50% calcium cetyl maleate.                                                           | 4                   | 1/2+           |
| 15      | +0.34% calcium $\alpha$ -eicosenylsuccinate.                                            | 4                   | 1/2            |
| 17      | +0.15% calcium cetyl sebacate.                                                          | 3 1/2 dil.          | 5 1/2+         |
| 20      | +0.61% calcium cetyl $\alpha$ -aminosuccinate.                                          | 4 1/2               | 1/2+           |
| 25      | +0.78% calcium cetyl malonate.                                                          | 4 1/2               | 1/2+           |
| 27      | +0.18% calcium $\alpha$ -cetenylysuccinate.                                             | 4                   | 1-             |
| 28      | +1.0% potassium cetyl oxalate.                                                          | 3 1/2+              | 0              |
| 29      | +0.10% calcium cetyl sebacate.                                                          | 7                   | 4              |
| 30      | +0.50% potassium $\alpha$ -cetylmalonate.                                               | 4 1/2               | 1 1/2          |
| 31      | +0.72% calcium cetyl fumarate.                                                          | 5                   | 1 1/2          |
| 32      | +0.50% calcium cetylphenate+0.40% calcium cetyl tartrate.                               | 8                   | 1+             |
| 34      | +0.50% calcium cetylphenate+0.50% calcium dicetyl citrate.                              | 7                   | 2 1/2+         |
| 35      | +0.50% calcium cetylphenate+0.50% calcium cetyl succinate.                              | 6                   | 1 1/2          |
| 39      | +0.50% calcium cetylphenate+0.50% calcium cetyl malate.                                 | 6                   | 1              |
| 40      | +0.50% calcium cetylphenate+0.50% calcium $\alpha$ -cetylmalonate.                      | 6                   | 1 1/2          |
| 41      | +0.50% calcium cetylphenate+0.50% calcium $\alpha$ -eicosenylsuccinate.                 | 7                   | 2 1/2+         |
| 42      | +0.50% calcium cetylphenate+0.50% calcium $\alpha$ -cetylphenate.                       | 6                   | 1 1/2          |
| 43      | +0.50% calcium cetylphenate+0.50% calcium $\alpha$ -cetylphenate.                       | 6                   | 1              |
| 44      | +0.50% calcium cetylphenate+0.50% calcium cetyl $\alpha$ -aminosuccinate.               | 7                   | 2 1/2+         |
| 45      | +0.50% calcium cetylphenate+0.50% calcium cetyl $\alpha$ -mercaptosuccinate.            | 6                   | 1 1/2          |
| 47      | +0.25% calcium cetylphosphate+0.40% calcium cetyl tartrate.                             | 7                   | 2 1/2          |
| 48      | +0.25% calcium cetylphosphate+0.50% calcium cetyl sebacate.                             | 4 1/2               | 1+             |
| 49      | +0.25% calcium cetylphosphate+0.18% calcium cetyl oxalate.                              | 5                   | 1 1/2          |
| 50      | +0.25% calcium cetylphosphate+0.18% calcium cetyl oxalate.                              | 5                   | 1 1/2          |
| 51      | +0.25% calcium cetylphosphate+0.50% calcium cetyl succinate.                            | 4                   | 1/2+           |
| 52      | +0.25% calcium cetylphosphate+0.50% calcium cetyl malate.                               | 4 1/2               | 1              |
| 53      | +0.25% calcium cetylphosphate+0.50% calcium $\alpha$ -cetylmalonate.                    | 4 1/2               | 1/2            |
| 54      | +0.25% calcium cetylphosphate+0.10% calcium $\alpha$ -cetenylysuccinate.                | 4                   | 1/2            |
| 55      | +0.25% calcium cetylphosphate+0.50% calcium dicetyl citrate.                            | 4 1/2               | 1-             |
| 57      | +0.25% calcium cetylphosphate+0.50% calcium $\alpha$ -eicosenylsuccinate.               | 5                   | 2-             |
| 58      | +0.50% calcium cetylphenate+0.25% calcium cetylphosphate+0.40% calcium cetyl tartrate.  | 8                   | 2+             |
| 59      | +0.50% calcium cetylphenate+0.25% calcium cetylphosphate+0.40% calcium dicetyl citrate. | 6                   | 1 1/2          |
| 60      | +0.50% calcium cetylphenate+0.25% calcium cetylphosphate+0.50% calcium dicetyl citrate. | 6                   | 2              |
| 61      | +0.50% calcium cetylphenate+0.25% calcium cetylphosphate+0.50% calcium cetyl succinate. | 4 1/2               | 1/2            |
| 62      | +0.50% calcium cetylphenate+0.25% calcium cetylphosphate+0.50% calcium cetyl malate.    | 6                   | 1-             |

TABLE III—Continued

| Example | Oil                                                                                                     | Color after heating | Color increase |
|---------|---------------------------------------------------------------------------------------------------------|---------------------|----------------|
| 62      | +0.50% calcium cetylphenate + 0.25% calcium cetylphosphate + 0.50% calcium cetyl maleate                | 6-                  | 1 1/2          |
| 63      | +0.50% calcium cetylphenate + 0.25% calcium cetylphosphate + 0.20% calcium $\alpha$ -cetenylysuccinate  | 5-                  | 1 1/2          |
| 64      | +0.50% calcium cetylphenate + 0.25% calcium cetylphosphate + 0.50% calcium $\alpha$ -eicosenylsuccinate | 7                   | 2 1/2          |
| 65      | +0.50% calcium cetylphenate + 0.25% calcium cetylphosphate + 0.15% calcium cetyl sebacate               | 6                   | 2              |
| 66      | +1.0% diisoamyl tartrate + 0.50% calcium diethyl citrate                                                | 4 1/2-              | 1              |
| 67      | +1.0% diisoamyl tartrate + 0.18% calcium cetyl oxalate                                                  | 7                   | 4              |
| 68      | +1.0% diisoamyl tartrate + 0.50% calcium cetyl succinate                                                | 6-                  | 2 1/2          |
| 69      | +1.0% diisoamyl tartrate + 0.50% calcium cetyl maleate                                                  | 4 1/2               | 1              |
| 70      | +1.0% diisoamyl tartrate + 0.50% calcium cetyl maleate                                                  | 4                   | 1 1/2          |
| 71      | +1.0% diisoamyl tartrate + 0.10% calcium $\alpha$ -centenylsuccinate                                    | 4 1/2               | 1              |
| 72      | +1.0% diisoamyl tartrate + 0.50% calcium $\alpha$ -eicosenylsuccinate                                   | 3 1/2               | 1 1/2          |
| 73      | +1.0% diisoamyl tartrate + 0.15% calcium cetyl sebacate                                                 | 3 dil.              | 4 1/2+         |

## EXAMPLES—SET IV

In many cases still further benefits may be derived from the incorporation of the metal salts of the invention to hydrocarbon oils, by reason of an enhanced "oiliness" and/or an increased load carrying capacity of the oils so compounded.

In the tests whose results are summarized in Table IV, the figures reported under "Weeks wear" are those obtained in the operation of a Weeks wear testing machine, in which a  $1\frac{1}{2}$  inch steel ball is pressed against a  $1\frac{1}{8}$  inch steel cylinder which is rotated at 600 R. P. M. and which dips into the oil being tested; the duration of the test is 16 hours and the body of oil is held at  $300^{\circ}$  F.; the results are reported in inches of wear  $\times 10^5$ , as measured on the cylinder. The figures reported under "Film strength" are those obtained in the operation of a Timken machine as described in the S. A. E. Journal, volume 28, page 53, 1928; the results are reported in pounds at failure.

TABLE IV  
Wear resistance and film strength

| Example | Oil                                                         | Weeks wear | Film strength |
|---------|-------------------------------------------------------------|------------|---------------|
| 4       | Western 30                                                  | 288        | 120           |
| 9       | +0.50% calcium cetyl tartrate                               | 74         | 160           |
| 11      | +0.18% calcium cetyl oxalate                                | 92         | 120           |
| 13      | +0.50% calcium cetyl maleate                                | 102        | 120           |
| 14      | +0.50% calcium cetyl maleate                                | 83         | 500           |
| 15      | +0.50% calcium $\alpha$ -cetylmalonate                      | 186        | 200           |
| 17      | +0.34% calcium $\alpha$ -eicosenylsuccinate                 | 143        | 160           |
| 25      | +0.20% calcium $\alpha$ -cetenylysuccinate                  | 106        | 220           |
| 35      | +0.50% calcium cetylphenate + 0.25% calcium diethyl citrate | 163        | 120           |
| B       | +1.0% aluminum dinaphthenate                                | 108        | 320           |
| D       | +0.50% calcium cetylphenate                                 | 639        | 120           |
|         |                                                             | 105        | 120           |

## EXAMPLES—SET V

Still further, the capability of hydrocarbon oils to absorb oxygen, when exposed thereto at su-

peratmospheric temperatures and pressures, is in many cases reduced or postponed by the incorporation in the oils of the metal salts of the invention, particularly those carrying a polar group of the character and in the position referred to repeatedly hereinabove.

In the tests whose results are reported in Table V, the oils referred to were subjected to the "oxidator test" particularly described in the Journal of Industrial and Engineering Chemistry, volume 28, page 26, 1936, at  $340^{\circ}$  F., which conditions may be noted as extremely severe. The results of the tests are reported in cubic centimeters of oxygen absorbed per 100 grams of the respective oils, at the periods of time indicated.

TABLE V  
Reduction of oxygen absorption

| Example | Oil                                            | Oxygen absorption |        |            |
|---------|------------------------------------------------|-------------------|--------|------------|
|         |                                                | 1 hr.             | 2 hrs. | 2 1/2 hrs. |
| 1       | Western 30                                     | 200               | 330    | 390        |
| 2       | +0.28% potassium cetyl tartrate                | 135               | 235    | 280        |
| 3       | +0.42% magnesium cetyl tartrate                | 80                | 200    | 270        |
| 4       | +0.57% aluminum cetyl tartrate                 | 87                | 150    | 175        |
| 5       | +0.50% calcium cetyl tartrate                  | 25                | 55     | 70         |
| 6       | +0.20% calcium cetyl maleate                   | 18                | 45     | 75         |
| 7       | +0.34% potassium cetyl citrate                 | 30                | 50     | 55         |
| 8       | +0.28% magnesium cetyl citrate                 | 35                | 135    | 190        |
| 9       | +0.52% aluminum cetyl citrate                  | 24                | 65     | 93         |
| 10      | +0.50% calcium diethyl citrate                 | 20                | 40     | 59         |
| 11      | +0.63% calcium $\alpha$ -eicosyltartrate       | 65                | 105    | 122        |
| 12      | +0.18% calcium cetyl oxalate                   | 35                | 80     | 145        |
| 13      | +0.50% calcium cetyl maleate                   | 22                | 60     | 90         |
| 14      | +0.50% calcium cetyl maleate                   | 75                | 150    | 260        |
| 15      | +0.50% calcium $\alpha$ -cetylmalonate         | 40                | 95     | 150        |
| 17      | +0.34% calcium $\alpha$ -eicosenylsuccinate    | 23                | 50     | 65         |
| 20      | +0.61% calcium cetyl $\alpha$ -aminoisocinate  | 20                | 50     | 60         |
| 21      | +0.78% calcium cetyl malonate                  | 190               | 275    | 310        |
| 26      | +0.25% calcium $\alpha$ -cetenylysuccinate     | 8                 | 30     | 47         |
| 31      | +0.10% calcium $\alpha$ -eicosylaminosuccinate | 100               | 240    | 290        |

50 Although we have no definitely acceptable theory to offer for the success of the compositions of the invention in preventing or retarding piston ring sticking and, with more particular respect to those compositions in which polar group sub-

55 stitution has been effected in the close proximity of the carbon atoms contained in the salt-forming carboxyl radical, in reducing oil corrosivity toward bearing metals, in stabilizing oil color at high temperatures, in reducing engine wear, in increasing oil film strength and in retarding oil

60 oxidizability at high temperatures, as well as in stabilizing in these and other ways oils already compounded with agents not of this invention, and do not, accordingly, wish to be limited by any theory which, at some more advanced stage in the development of the art, might prove questionable or untenable, we nevertheless wish to point out, in connection with the examples above

65 and the few typical structural representations below, the manner in which the results brought about by the practice of the invention are considered by us now to be attributable to the position occupied by the designated polar groups, with respect to the salt-forming carboxyl group of the molecule.

TABLE VI

Structures, with particular relation to polar groups

| Example |                                         | Structure                                                                                                                                                                                                                                                            |
|---------|-----------------------------------------|----------------------------------------------------------------------------------------------------------------------------------------------------------------------------------------------------------------------------------------------------------------------|
| 1.....  | Potassium alkyl tartrate.....           | $\text{ROOC}-\text{HCOH}-\text{HCOH}-\text{COOK}$                                                                                                                                                                                                                    |
| 2.....  | Magnesium alkyl tartrate.....           | $(\text{ROOC}-\text{HCOH}-\text{HCOH}-\text{COO})_2\text{Mg}$                                                                                                                                                                                                        |
| 3.....  | Aluminum alkyl tartrate.....            | $(\text{ROOC}-\text{HCOH}-\text{HCOH}-\text{COO})_2\text{Al}(\text{OH})$                                                                                                                                                                                             |
| 5.....  | Calcium alkyl malate.....               | $(\text{ROOC}-\text{HCOH}-\text{HCOH}-\text{HCOH}-\text{COO})_2\text{Ca}$                                                                                                                                                                                            |
| 7.....  | Magnesium alkyl citrate.....            | $\begin{array}{c} \text{H}_2\text{C}-\text{COOR} \quad \text{ROOC}-\text{CH}_2 \\   \quad \quad \quad   \\ \text{HOC}-\text{COOR} \quad \text{ROOC}-\text{COH} \\   \\ \text{H}_2\text{C}-\text{COO}-\text{Mg}-\text{OOC}-\text{CH}_2 \end{array}$                   |
| 8.....  | Aluminum alkyl citrate.....             | $\begin{array}{c} \text{H}_2\text{C}-\text{COOR} \quad \text{ROOC}-\text{CH}_2 \\   \quad \quad \quad   \\ \text{HOC}-\text{COOR} \quad \text{ROOC}-\text{COH} \\   \\ \text{H}_2\text{C}-\text{COO}-\text{Al}-\text{OOC}-\text{CH}_2 \\   \\ \text{OH} \end{array}$ |
| 10..... | Calcium $\alpha$ -eicosyltartrate.....  | $\begin{array}{c} \text{COO} \\   \\ \text{H}_2\text{C}_{18}-\text{C}-\text{C}-\text{COH} \\   \quad   \\ \text{H} \quad \text{H} \\   \\ \text{COO} \end{array} \text{Ca}$                                                                                          |
| 11..... | Calcium alkyl oxalate.....              | $\begin{array}{c} \text{ROOC} \quad \text{COOR} \\   \quad   \\ \text{COO}-\text{Ca}-\text{OOC} \end{array}$                                                                                                                                                         |
| 12..... | Calcium alkyl succinate.....            | $\begin{array}{c} \text{ROOC} \quad \text{COOR} \\   \quad   \\ \text{CH}_2 \quad \text{CH}_2 \\   \quad   \\ \text{CH}_2 \quad \text{CH}_2 \\   \quad   \\ \text{COO}-\text{Ca}-\text{OOC} \end{array}$                                                             |
| 13..... | Calcium alkyl malate.....               | $\begin{array}{c} \text{ROOC} \quad \text{COOR} \\   \quad   \\ \text{HCOH} \quad \text{HOCH} \\   \quad   \\ \text{HCH} \quad \text{HCH} \\   \quad   \\ \text{COO}-\text{Ca}-\text{OOC} \end{array}$                                                               |
| 14..... | Calcium alkyl maleate.....              | $\begin{array}{c} \text{ROOC} \quad \text{COOR} \\   \quad   \\ \text{CH} \quad \text{HC} \\   \quad   \\ \text{CH} \quad \text{HC} \\   \quad   \\ \text{COO}-\text{Ca}-\text{OOC} \end{array}$                                                                     |
| 15..... | Calcium $\alpha$ -alkylmalonate.....    | $\begin{array}{c} \text{COO} \\   \\ \text{R}-\text{CH}-\text{Ca} \\   \\ \text{COO} \end{array}$                                                                                                                                                                    |
| 16..... | Calcium $\alpha$ -cetenylsuccinate..... | $\begin{array}{c} \text{COO} \\   \\ \text{H}_2\text{C}_{14}-\text{C}=\text{C}-\text{CH} \\   \quad   \\ \text{H} \quad \text{H} \\   \\ \text{CH}_2 \\   \\ \text{COO} \end{array} \text{Ca}$                                                                       |
| 18..... | Calcium alkyl sebacate.....             | $\begin{array}{c} \text{ROOC} \quad \text{COOR} \\   \quad   \\ (\text{CH}_2)_8 \quad (\text{CH}_2)_8 \\   \quad   \\ \text{COO}-\text{Ca}-\text{OOC} \end{array}$                                                                                                   |
| 21..... | Calcium alkyl malonate.....             | $\begin{array}{c} \text{ROOC} \quad \text{COOR} \\   \quad   \\ \text{CH}_2 \quad \text{H}_2\text{C} \\   \quad   \\ \text{COO}-\text{Ca}-\text{OOC} \end{array}$                                                                                                    |

The above few typical representations will suffice to enable all of the earlier and numerous additional individual members of the agents contemplated for incorporation in the compositions of the invention to be studied in connection with their above exemplified effects when so incorporated.

In consideration of the effects as exemplified and in view of the structures as indicated, it is permissible to generalize briefly as follows: While all of the agents of the invention are effective to prevent such deterioration as is evidenced

by piston ring sticking, they differ considerably among themselves with respect to the degree of their capabilities to retard other types of deteriorations, as for example corrosivity toward bearing metals, retardation or inhibition of corrosivity brought about by the additional presence of another type of compounding agent, suppression of the formation of color bodies, and the like. It is believed, at the present state of our knowledge of these phenomena, that the presence of a polar group additional to the salt-forming carboxylic acid group, such as  $-\text{COOH}$ ,

—OH, —COOR, —NH<sub>2</sub>, and the like, as above listed and exemplified, in a position in close proximity to the carbon atom of the salt-forming carboxylic acid radical, is the means by which these highly beneficial effects are brought about, and that the effectiveness of the polar group or groups decreases as their distance from the salt-forming carboxyl radical increases. It must be noted, however, that the polar group or groups so present or introduced must not be capable of splitting out, to form a corrosive acidic substance, and such groups as —Cl, —Br, —I, —F, —OSO<sub>2</sub>OR, and —OSO(OR) are accordingly not contemplated as within the designation of polar group or radical as the same is employed herein for the purposes of this invention.

Generally, measurable improvements in the properties of hydrocarbon oils are obtained by the incorporation of as little as 0.1% of the agents of the invention, but amounts between about 0.2% and 2.0% of the agents, by weight based on the oil, are preferable, dependent upon the degree of inherent tendency toward degradation of the oil itself or as otherwise compounded; amounts higher than about 5.0% are regarded as unnecessary in the best practice of the invention.

A feature of the invention is in the preparation and distribution of bases or concentrates containing relatively large proportions of the additive agents in admixture with hydrocarbon oils of the lubricating or less viscous types or, if more suitable in conjunction with certain of the agents, by reason of solubility relationships or the like, in admixture with aromatic hydrocarbons or with alcohols, esters, ketones or ethers, generally of the aliphatic series. Admixtures of the agents and lubricating oils or other solvents or carriers containing upward of 50% of the essential agents, by weight, may be thus prepared and distributed, for later blending with the particular lubricating oil media desired to be put to use, as occasion demands. In the preparation of either the finished oils of the invention or the bases or concentrates referred to, complete or clear and homogeneous solution is not always necessary: blending agents or homogenizers may be employed if desirable, to prevent sedimentation of the more oil-insoluble of the agents, but it has been found the possible detrimental effect of the presence of filterable insoluble materials of this character, if indeed present, is determined largely by the particular conditions attending the contemplated use, and that their presence is not in all cases deleterious to the functioning of the compositions in their intended manner.

While the character of the invention has been given in detail and numerous illustrative examples of the preparation and utility of the compositions of the invention have been described, this has been done largely by way of illustration and with the intention that no limitation should be imposed upon the invention thereby. It will be obvious to those skilled in the art that numerous modifications and variations of the above illustrative examples may be effected in the practice of the invention, which is intended to be of the scope of the appended claims.

We claim:

1. A liquid hydrocarbon oil of the lubricating oil class, normally tending to deteriorate at operating temperatures encountered in the lubrication of internal combustion engines, containing dissolved in the oil a small amount, sufficient

to retard the said deterioration, of an oil-soluble metal salt of an acid of the type



5 in which *n* is a whole number and in which hydrocarbon radicals may replace one or more of the hydrogen atoms of the —CH<sub>2</sub>— groups, and in which at least two polar radicals have been substituted for hydrogen atoms carried by carbon atoms other than that of the salt-forming carboxylic acid group.

10 2. A liquid hydrocarbon oil of the lubricating oil class, normally tending to deteriorate at operating temperatures encountered in the lubrication of internal combustion engines, containing dissolved in the oil a small amount, sufficient to retard the said deterioration, of an oil-soluble metal salt of an acid of the type



20 in which *n* is a whole number greater than 1 and in which hydrocarbon radicals may replace one or more of the hydrogen atoms of the —CH<sub>2</sub>— groups, and in which at least two polar radicals have been substituted for hydrogen atoms carried by carbon atoms at least one of which is placed not farther than the gamma position relative to the carbon atoms of the salt-forming carboxylic acid group.

25 30 3. A liquid hydrocarbon oil of the lubricating oil class, normally tending to deteriorate at operating temperatures encountered in the lubrication of internal combustion engines, containing an oil-soluble metal salt of an acid of the type

35  $\text{HOOC}-(\text{CH}_2)_n-\text{COOH}$ , in which *n* is a whole number greater than 1 and in which hydrocarbon radicals may replace one or more of the hydrogen atoms of the —CH<sub>2</sub>— groups, and in which at least two polar radicals have been substituted

40 45 for hydrogen atoms carried on carbon atoms at least one of which is placed not farther than the gamma position relative to the carbon atom of the salt-forming carboxylic acid group, the said polar radicals being incapable of forming a corrosive acidic product when split out from the said position upon exposure to superatmospheric temperatures in the presence of the hydrocarbon oil, said metal salt being dissolved in the oil in small amount sufficient to retard the said deterioration.

50 55 4. A liquid hydrocarbon oil of the lubricating oil class, normally tending to deteriorate at operating temperatures encountered in the lubrication of internal combustion engines, containing a small amount, sufficient to retard the said deterioration, of a polyvalent metal salt of a partially-esterified acid of the type



60 in which *n* is a whole number, and in which at least one —OH and at least one other polar radical are substituted for hydrogen atoms of the said —(CH<sub>2</sub>)— groups.

65 5. A liquid hydrocarbon oil of the lubricating oil class, normally tending to deteriorate at operating temperatures encountered in the lubrication of internal combustion engines, containing a small amount, sufficient to retard the said deterioration, of a polyvalent metal salt of a partially-esterified citric acid.

70 6. A liquid hydrocarbon oil of the lubricating oil class, normally tending to deteriorate at operating temperatures encountered in the lubrication of internal combustion engines, containing a small amount, sufficient to retard the said deterioration, of a polyvalent metal salt of a tar-

taric acid in which one carboxyl group is esterified.

7. An improved liquid hydrocarbon composition comprising a major proportion of hydrocarbon lubricating oil subject to deterioration at operating temperatures encountered in the lubrication of internal combustion engines and a minor proportion, sufficient to inhibit said deterioration, of a metal salt of an aliphatic polycarboxylic acid having at least two carboxyl groups and at least two additional polar groups on alkyl carbon atoms at least one of which is not farther than the gamma position relative to a carboxyl group of said acid, said acid having no more than eight alkyl carbon atoms between the nearest two carboxyl groups thereof and containing an oil-solubilizing substituent.

8. An additive for lubricants capable of inhibiting deterioration of a hydrocarbon oil at operating temperatures encountered in the lubrication of internal combustion engines, comprising a concentrated solution in a viscous oil of an oil-soluble metal salt of an aliphatic polycarboxylic acid having at least two carboxyl groups and at least two additional polar groups on alkyl carbon atoms at least one of which is not farther than the gamma position relative to a carboxyl group of said acid, said acid having no more than eight alkyl carbon atoms between the nearest two carboxyl groups thereof and containing an oil-solubilizing substituent, said solution being capable of dilution with mineral lubricating oil to form a homogeneous mixture containing from approximately 0.1% to 2% by weight of the salt based on the total amount of lubricating oil.

9. A liquid lubricating oil composition comprising a hydrocarbon oil in major part; about 0.1 to 5% by weight based on the hydrocarbon oil and sufficient to inhibit corrosiveness of the finished oil toward bearing metal alloys of the type of copper-lead and cadmium-silver alloys of a metal salt of an acid of the type



in which  $n$  is a whole number from 1 to 8 inclusive, in which at least two of the hydrogen

atoms of the  $-\text{CH}_2-$  groups are replaced by polar groups and in which one or more hydrogen atoms of the  $-\text{CH}_2-$  groups may be replaced by hydrocarbon radicals; and about 0.1 to 5% by weight based on the hydrocarbon oil of a metal salt selected from the group consisting of metal alcoholates and metal phenates.

10. The oil of claim 9, wherein the first named metal salt is a polyvalent metal salt and the second named metal salt is an oil-soluble polyvalent metal phenate.

11. The oil of claim 9, wherein the first named metal salt is a polyvalent metal salt and the second named metal salt is an oil-soluble alkaline earth metal salt of an alkylated phenol.

12. A liquid hydrocarbon oil of the lubricating oil class, normally tending to deteriorate at operating temperatures encountered in the lubrication of internal combustion engines, containing a small amount, sufficient to retard the said deterioration, of a polyvalent metal salt of a half ester of mucic acid.

13. A lubricating oil comprising, as the major ingredient, a petroleum lubricating oil and containing about 0.1 to 5 per cent by weight based on finished oil of an oil-soluble alkaline earth metal salt of a partially esterified citric acid.

14. The oil of claim 13, wherein said alkaline earth metal is calcium.

15. A lubricating oil comprising, as the major ingredient, a petroleum lubricating oil and containing about 0.1 to 5 per cent by weight based on finished oil of an oil-soluble alkaline earth metal salt of a partially esterified tartaric acid.

16. The oil of claim 15, wherein said alkaline earth metal is calcium.

17. A lubricating oil comprising, as the major ingredient, a petroleum lubricating oil and containing about 0.1 to 5 per cent by weight based on finished oil of an oil-soluble alkaline earth metal salt of a partially esterified mucic acid.

18. The oil of claim 17, wherein said alkaline earth metal is calcium.

BRUCE B. FARRINGTON.

JAMES O. CLAYTON.

DORR H. ETZLER.